

1

3,105,818

### LUBRICATING COMPOSITIONS

William A. Hewett, Oakland, Calif., assignor to Shell Oil Company, a corporation of Delaware  
No Drawing. Filed June 2, 1959, Ser. No. 817,462

4 Claims. (Cl. 252—47.5)

This invention relates to lubricants and particularly to highly detergent lubricants useful under severe operating conditions, such as under extreme high speed and at high temperatures, and to a new and novel class of polymeric additives therefor.

It is well known that the high pressure occurring in certain types of gears and bearings may cause rupture of lubricant films with consequent damage to the machinery. It is known that various base lubricants can be improved in their protective properties of rubbing surfaces by the addition of certain substances, so-called extreme pressure agents, so that excessive wear, scuffing and seizure are minimized or prevented.

It is known that certain compounds of metal-reactive elements, such as certain compounds of chlorine, sulfur and phosphorus, as well as certain other compounds, such as some compounds of lead, impart extreme pressure properties to various lubricants. Notable among the substances heretofore used are the lead soaps, phosphoric acid esters, free or bound sulfur and certain chlorinated organic compounds. A principal objection to many of these extreme pressure agents is their lack of detergency and their high reactivity with the metallic surface, causing etching, corrosion and discoloration of the metal surface. Another objection to chemically reactive extreme pressure agents is that they alter the original chemical nature of the contacting surface, which under certain conditions is undesirable. Additionally, because of the activity of agents of this type, they usually are depleted rapidly resulting in only a temporary solution to the problem of extreme pressure lubrication.

It has now been discovered that improved detergent and extreme pressure lubricants are provided by a suitable lubricating oil containing oil-soluble high molecular weight non-ash halo-mercapto-containing polymeric compounds having essentially a long linear hydrocarbon backbone chain and attached thereto in a uniform or random fashion two kinds of essential groups, one an oil-solubilizing hydrocarbyl radical, preferably an alkyl radical having an average of between 8 and 20 carbon atoms (preferably 10-16) bonded directly to the hydrocarbon backbone chain or indirectly thereto through a polar group and the other an alkyl radical containing a halogen and an aryl mercapto group on adjacent carbons of the alkyl radical, which groups are at least two carbon atoms removed from the main hydrocarbon polymer chain alkyl carbons. This polar substituted radical is represented by the formula



where Q is an aryl radical, X is a polar radical such as halogen, amino, nitro, sulfo or the like, x and y are integers of at least 1, preferably 4-20, and z is a number

2

from zero to 2. The number of units (I) in the final polymer can vary from 10 to 1000 or more, preferably from 100 to 800, inclusive. Polymers of this invention contain a plurality of units represented by



where x, y, z, Q and X are as defined, m is a whole number, and Y is an oil-solubilizing radical containing a  $\text{C}_{8-20}$  alkyl radical attached directly or indirectly to the main backbone chain through a polar group such as



where Z is hydrogen or an alkyl radical. The molecular weight of the polymer varies from about a thousand to about a million, preferably from 10,000 to 500,000.

The oil-soluble halo-mercapto aryl containing polymers of the above type are prepared by reacting aryl sulfenyl halides with an oil-soluble unsaturated linear hydrocarbon polymer which, in turn, is prepared by polymerizing a polyene hydrocarbon with a monoolefinically polymerizable monomer having a long-chain alkyl radical such as long-chain alpha-olefins, long chain alkyl esters of alpha,beta-unsaturated acids, such as esters of acrylic and methacrylic acids, esters of lower unsaturated alcohols, such as vinyl and allyl alcohol esters of long chain fatty acids and long chain N-alkyl unsaturated fatty acid amides such as N-alkyl acrylamides.

The sulfenyl halides useful in the preparation of the novel polymers of this invention include aryl sulfenyl halides, such as benzene sulfenyl chloride, bromide, iodide or fluoride, e.g., benzene sulfenyl chloride, p-toluene sulfenyl chloride, butyl benzene sulfenyl chloride, etc.; halogen-substituted benzene sulfenyl halides, e.g., chlorobenzene sulfenyl chloride, 2,3-, 3,4- or 2,4-dibromobenzene sulfenyl chloride, 2,4,6-trichlorobenzenesulfenyl chloride, pentachlorobenzene sulfenyl chloride, 2-chloro-3-bromobenzenesulfenyl chloride, p-fluorobenzenesulfenyl chloride, etc.; and nitro-substituted benzenesulfenyl halides such as p-nitrobenzene sulfenyl chloride or 2,4-dinitrobenzenesulfenyl chloride or bromide, etc. There may also be used benzene sulfenyl halides such as 4-chloro-2-nitrobenzene sulfenyl chloride, 2-chloro-4-nitrobenzene sulfenyl chloride, or 2-chloro-5-methylbenzenesulfenyl chloride, i.e., benzenesulfenyl halides having a diversity of substituents in the benzene ring. Especially preferred in the present process are the chloro- and/or nitro-substituted benzene sulfenyl halides.

Suitable polyene hydrocarbons for forming the copolymers are  $\text{C}_{4-20}$  dienes, for example, 1,3- and 1,4-pentadiene, isoprene, 1,3-hexadiene, 1,3,5-heptatriene, 1,3-cyclopentadiene, methylcyclopentadiene, 1,3- and 1,4-cyclohexadiene, methylcyclohexadiene, and mixtures thereof. Other dienes are obtained by dehydration of unsaturated

fatty alcohols such as lauroylel, myristoleyl, palmitoleyl, gadoleyl, linoleyl, ricinoleyl alcohols. A diene of this type which is particularly suitable is obtained by dehydrating oleyl alcohol which results in a 50-50 mixture of monoenes and dienes of  $C_{12}$  to  $C_{20}$  carbon atoms having the following properties:

|                                  |                                                             |
|----------------------------------|-------------------------------------------------------------|
| Iodine value                     | 183.                                                        |
| Hydroxyl value                   | 0.4.                                                        |
| Boiling range                    | Over 100° C. at 1 mm. Hg.                                   |
| Appearance                       | Colorless-pale yellow liquid.                               |
| Melting range                    | -55 to 70° C. (approx.).                                    |
| Flash point (Cleveland open cup) | 152° C.                                                     |
| Viscosity                        | 2.47 centistokes at 100° F.,<br>1.29 centistokes at 210° F. |
| Specific gravity, 25/25° C.      | 0.7965.                                                     |

This material will be identified as "Compound A."

Representative oil-solubilizing monomer compounds which are used to form the copolymers with the polyene hydrocarbons include alpha-unsaturated long chain hydrocarbons, unsaturated esters, unsaturated amides, e.g., such as decene-1, dodecene-1, tridecene-1, tetradecene-1, hexadecene-1, heptadecene-1, octadecene-1, tritriacontene-1, tetratriacontene-1, heptacontene-1, 4-methyl-decene-1, 4, 4-dimethyl-decene-1, 5,5-dimethylhexene-1, 5,5,7,7-tetramethyl-decene-1, 4,4,6,6-tetramethylheptene-1, etc., vinyl decanoate, vinyl laurate, vinyl tridecanoate, vinyl myristate, vinyl pentadecanoate, vinyl palmitate, vinyl margarate, vinyl stearate, vinyl nonadecanoate, vinyl arachidate, vinyl behenate, vinyl 4,5,6-trimethyldecanoate, vinyl 6,8,9-triethyl tridecanoate, vinyl 12-hydroxystearate, vinyl 9,10-dihydroxystearate, vinyl chlorostearate, vinyl cyano-stearate, vinyl acetylstearate, vinyl dodecyl ether, vinyl tridecyl ether, vinyl tetracosyl ether, vinyl hexacosyl ether, allyl stearate, allyl dodecyl ether, N-lauryl methacrylamide, N-stearyl methacrylamide, N,N-distaryl methacrylamide, lauryl methacrylate, stearyl methacrylate and mixtures thereof.

The mol ratio of the polyene hydrocarbon to the oil-solubilizing monomer compound can be varied within relatively wide limits, e.g., from 1/10 to 10/1, preferably from 1/5 to 5/1, respectively. The polymer (prior to treatment with an aryl sulfenyl halide compound) should have a substantial amount of unsaturation.

Depending on the monomers used the polymers can be prepared thermally or in the presence of a suitable catalyst. Thus, with monomers such as butadiene, isoprene, "Compound A" and long chain alpha-olefins such as alpha-dodecene or alpha-octadecene, the so-called Ziegler catalysts are preferred, such as combinations of aluminum trialkyls and a variable valence metal compound, e.g., titanium tetrachloride. In the formation of other types of oil-soluble polymers such as copolymers of the polyene (e.g., butadiene, isoprene, or "Compound A") with lauryl methacrylate or with vinyl stearate or with N-lauryl methacrylamide, oxygen-yielding catalysts are preferred such as, for example, various organic peroxides, including aliphatic, aromatic, heterocyclic and acyl peroxides, such as diethyl peroxide, tertiary butyl hydroperoxide, dibenzoyl peroxide, dimethylthienyl peroxide, dicyclohexyl peroxide, dilauroyl peroxide and urea peroxide. These are mentioned by way of non-limiting examples of suitable organic peroxides. Other catalysts include sodium bisulfite, diethyl sulfoxide, ammonium persulfate, alkali metal perborates, azo compounds, such as alpha-alpha-azodiisobutyronitrile, etc.

The following Examples I-X are given as representative preparations of the intermediate copolymers for reaction with sulfenyl halide compounds to form the desired end product.

#### Example I

About 0.66 mole of 1-octadecene, 1.33 moles of 1-dodecene and 0.5 mole of "Compound A" in cyclohexane were reacted in the presence of a Ziegler catalyst

$(C_2H_5)_3Al\cdot TiCl_4$  at room temperature for about 24 hours. The catalyst was destroyed by addition of methanol and polymer thereafter purified by benzene washing and precipitating from alcohol and vacuum drying. The polymer had an average molecular weight of 300,000 and an average of 750 double bonds per polymer molecule as shown by bromine number.

#### Example II

About 0.5 mole of "Compound A," 0.17 mole of 1-tetradecene and 0.34 mole of 1-dodecene in benzene were reacted in the presence of the Ziegler catalyst and under the conditions of Example I. The polymer formed had a molecular weight between 350,000-400,000 and a bromine number of 50.

#### Example III

About 2 moles of pentadiene and 1 mole of lauryl methacrylate and 1% diterbutyl peroxide were reacted at 75-100° C. for about 24 hours. The polymer was purified by alcohol washing, filtered and dried. The resulting copolymer had a molecular weight of 3000-5000 and substantial unsaturation as shown by a bromine number of 80 to 100.

Following essentially the procedures of Examples I-III, other polymers were prepared in accordance with the following tabulation:

| Example | Catalyst               | Temperature, °C. | Polyene/oil-soluble mono-olefins ratio                                                                    |
|---------|------------------------|------------------|-----------------------------------------------------------------------------------------------------------|
| IV      | Ziegler Cat.           | Room temp.       | butadiene(2)/octadecene-1 (1).                                                                            |
| V       | do                     | 60-70            | isoprene(2)/octadecene-1 (1).                                                                             |
| VI      | Benzoyl peroxide.      | 80               | isoprene(3)/lauryl methacrylate(1).                                                                       |
| VII     | do                     | 110              | butadiene(2)/ $C_{14-18}$ diene of dehydrated $C_{14-18}$ unsaturated fatty alcohol(1)/vinyl stearate(1). |
| VIII    | Diterb-butyl-peroxide. | 80               | pentadiene (3)/N-lauryl-methacrylamide (1).                                                               |
| IX      | do                     | 120              | Diene of ricinoleyl alcohol (3)/lauryl methacrylate (1) stearylmethacrylate (1).                          |
| X       | do                     | 100              | Diene of linoleyl alcohol(3)/allyl stearate(1).                                                           |

The final oil-soluble polymeric additive is prepared by reacting the unsaturated copolymer, such as those of Examples I-X, with one or more of the sulfenyl halide compounds by any suitable means, such as described in Jour. Am. Chem. Soc., 75, 6030 (1953) or 78, 1201 (1958). Specifically, in carrying out the final reaction the sulfenyl halide is simply contacted with the unsaturated polymer at ordinary, increased or decreased temperatures, until formation of the halo-sulfur containing product has occurred. Depending upon the individual reactants employed, as well as on the quantities used, heating or cooling of the reactant mixture may be required. In many cases, formation of the products takes place spontaneously, although the reaction may, if desired, be expedited by heating the reaction temperature and in dissipating the heat of reaction. Useful inert solvents and diluents are, e.g., benzene, toluene, hexane, ether, etc. An excess of either reactant and gradual introduction of the other may also result in smoother operation. The present reaction may also be effected at increased or decreased pressure, or in the presence of a catalyst; however, the ease of reaction at ordinary atmospheric pressure and in the absence of catalysts generally requires no control of the reaction by pressure variation or acceleration thereof by catalytic means.

The invention is further illustrated, but not limited, by the following examples:

#### Example A

In a suitable vessel 40 grams of the copolymer of Example II was dissolved in 200 ml. of benzene under a nitrogen atmosphere with stirring. To the mixture was

added 30 grams of 2,4-dinitrobenzene sulfenyl chloride and the mixture was stirred at room temperature for about 72 hours. The chlorine-sulfur-containing polymer was then precipitated from solution with methanol and then dissolved in benzene, filtered, precipitated with methanol and the procedure repeated. The polymer was then vacuum oven dried at 0.1 mm., 120° C. to give a polymer product having a plurality of beta-chloroalkyl 2,4-dinitrophenyl sulfide units having the following analysis:

|                      |      |
|----------------------|------|
| Percent wt. carbon   | 74.9 |
| Percent wt. hydrogen | 11.6 |
| Percent wt. nitrogen | 2.35 |
| Percent wt. chlorine | 3.01 |
| Percent wt. sulfur   | 2.71 |

### Example B

The procedure of Example A was followed using the polymer of Example II and benzene sulfenyl chloride as the sulfenyl halide compound. The final polymer molecule contained over 500 units of



groups distributed in the molecule.

### Example C

The procedure of Example A was followed using the polymer of Example I and 2,4-dinitrobenzene sulfenyl chloride. The final product contained over 500 units of



groups distributed in the molecule.

Following essentially the above procedures other polymers containing a plurality of halogen-sulfur-containing groups in the molecule were prepared in accordance with the following tabulation.

| Example | Polymer | Functional Group Introduced                                                                                 |
|---------|---------|-------------------------------------------------------------------------------------------------------------|
| D       | Ex. III | -Cl<br>-C <sub>4</sub> H <sub>9</sub><br>-S-C <sub>6</sub> H <sub>4</sub> -NO <sub>2</sub>                  |
| E       | Ex. V   | -Br<br>-S-C <sub>6</sub> H <sub>4</sub> -Cl<br>-NO <sub>2</sub>                                             |
| F       | Ex. VI  | -Cl<br>-S-C <sub>6</sub> H <sub>4</sub> -NO <sub>2</sub>                                                    |
| G       | Ex. IX  | -Cl<br>-C <sub>6</sub> H <sub>4</sub> -NH <sub>2</sub><br>-S-C <sub>6</sub> H <sub>4</sub> -NH <sub>2</sub> |
| I       | Ex. X   | -Cl<br>-C <sub>6</sub> H <sub>4</sub> -Cl<br>-S-C <sub>6</sub> H <sub>4</sub> -NO <sub>2</sub>              |

The halo-sulfur-containing polymers are oil-soluble and

are used in amounts of from about 0.5% to about 20%, preferably from about 1% to about 5% by weight. However, under certain storage and use conditions, it is desirable to incorporate into oil compositions containing these polymers a small amount (0.1-10%) of an oil-soluble branched-chain aliphatic monohydric alcohol. These alcohols can effectively stabilize such compositions without destroying the extreme pressure properties of such oil compositions.

The lubricating oil base is suitably selected from various synthetic oils or natural hydrocarbon oils having a viscosity range of from 50 SUS at 100° F. to 250 SUS at 210° F. (SAE viscosity number ranging from SAE 5W to SAE 90). The natural hydrocarbon oils are obtainable from paraffinic, naphthenic, asphaltic or mixed base crudes, and/or mixtures thereof. Useful synthetic oils include polymerized olefins, alkylated aromatics, isomerized waxes, copolymers of alkylene glycols and alkylene oxide (Ucon fluid, U.S. 2,425,755, 2,425,845 and 2,774,733) organic polyesters such as esters of an aliphatic dibasic acid and a monohydric alcohol, such as di-2-ethyl hexyl sebacate or di-2-ethyl hexyl adipate esters of polyhydric alcohols and monocarboxylic acids, such as pentaerythritol tetracaproate, and the like. Useful Ucon fluids are Ucon 50HB170, Ucon 50HB660 or Ucon LB550X, which are copolymers of ethylene and 1,2-propylene oxides; the diols as well as their mono- and dialkyl ethers are useful. The hydrocarbon oils may be blended with fixed oils such as castor oil, lard oil and the like and/or synthetic oils as mentioned or silicone polymers and the like. Typical oils of this type are petroleum motor oils (A) and (B), characterized below, (A) being paraffinic in character and (B) naphthenic in character:

| Properties                | (A)<br>(SAE 10W) | (B)<br>(SAE 30) |
|---------------------------|------------------|-----------------|
| Pour point, ° F.          | -10              | -5              |
| Flash, ° F.               | 390              | 415             |
| Viscosity, SUS at 210° F. | 44               | 58              |
| Viscosity Index           | 90               | 60              |

Other suitable oils are specification gas turbine lube oils having the following properties:

| Grade                     | 1010 | 1065 |
|---------------------------|------|------|
| Flash, COC, ° F.          | 300  | 465  |
| Pour, ° F.                | -10  | 0    |
| Viscosity, SUS at 100° F. | 59.4 | 530  |
| Neutral Number            | 0.02 | 0.01 |
| Ash                       | None | None |

The following compositions are illustrative of the invention, the percentages being by weight.

| Composition A:       | Percent |
|----------------------|---------|
| Example A additive   | 2       |
| 1010 mineral oil     | Balance |
| Composition B:       |         |
| Example B additive   | 2       |
| 1010 mineral oil     | Balance |
| Composition C:       |         |
| Example C additive   | 2       |
| 1010 mineral oil     | Balance |
| Composition D:       |         |
| Example A additive   | 5       |
| Mineral oil (SAE 90) | Balance |
| Composition E:       |         |
| Example D additive   | 1       |
| 1010 mineral oil     | Balance |
| Composition F:       |         |
| Example E additive   | 3       |
| SAE 90 mineral oil   | Balance |
| Composition G:       |         |
| Example F additive   | 2       |
| SAE 90 mineral oil   | Balance |

## Composition I:

|                                                                                            |         |
|--------------------------------------------------------------------------------------------|---------|
| Example A additive.....                                                                    | 5       |
| Ucon 50HB660 (polyethylene propylene glycol having a SUS viscosity at 100° F. of 660)..... | Balance |
|                                                                                            | 5       |

## Composition J:

|                               |         |
|-------------------------------|---------|
| Example A additive.....       | 5       |
| Di-2-ethylhexyl sebacate..... | Balance |

Compositions of this invention and other compositions were evaluated for their ability to impart to mineral oil (1) detergency as determined by the Carbon Black Dispersion Test described in the Journal of Colloid Science, vol. 12, October 1957, No. 5, pages 500-522; at 100° C. and 5 r.p.m.; and (2) extreme pressure properties as determined in the spur gear machine. The results are shown in Table I.

The spur gear machine consists essentially of two geometrically similar pairs of gears connected by two parallel shafts. The gear pairs are placed in separate gear boxes, which also contain the supporting ball bearings. One of the shafts consists of two sections connected by a coupling. Loading is accomplished by locking one side of the coupling and applying torque to the other. The conditions of the test were:

Speed ..... 3200  
 Oil temperature ..... ° F. 100  
 Oil flow-rate ..... cc./sec. 10  
 Load in increments, 5 min. at each setting.

TABLE I

| Compositions                                                             | Deflocculating Ability, ohms | Score Load, No./in. |
|--------------------------------------------------------------------------|------------------------------|---------------------|
| (1) Composition A                                                        | $12 \times 10^3$             | 12,000              |
| (2) Mineral oil (1010)+2% mixed $C_{8-18}$ alkyl methacrylate copolymer. | $3 \times 10^3$              | 700                 |
| (3) Mineral oil (1010)+2% neutral Ca petroleum sulfonate.                | $3.3 \times 10^3$            | 600                 |
| (4) Mineral oil (1010).....                                              | $3 \times 10^3$              | 600                 |

The polymers of this invention are useful also for providing superior load-carrying properties in lubricating oils which contain minor amounts of other agents which are non-reactive with the polymer, such as silicone anti-foaming agents, alkylphenol anti-oxidants, polyacrylate ester viscosity-index improvers, and the like.

I claim as my invention:

1. A lubricating oil composition comprising a major amount of mineral oil and from about 0.5% to 20% of an oil-soluble linear hydrocarbon polymer containing units of  $C_{8-20}$  alkyl groups and



groups attached to different carbons of the linear hydrocarbon chain where Q is benzene, X is a polar group selected from the group consisting of halogen, amino, nitro

and sulfo groups, the number of halo and  $\text{S} \text{ ---} \text{Q} \text{ ---} \text{X}_2$  units in the polymer varying from 10 to 1000, and x and y are integers of at least 1, and z is a number from 0 to 2, the molecular weight of the polymer ranging from 10,000 to 500,000.

2. A mineral lubricating oil composition comprising a major amount of mineral lubricating oil and from about 1% to about 5%, of an oil-soluble linear hydrocarbon polymer containing  $C_{8-20}$  alkyl groups and Cl,



groups on different carbon atoms of the linear hydrocarbon chain with the latter two groups, the number of such groups in the polymer ranging from 100 to 800 units and being attached to adjacent carbon atoms of an alkyl side chain and X is selected from the group consisting of chlorine and nitro group, the molecular weight of the polymer being from 10,000 to 500,000.

3. A mineral lubricating oil composition comprising a major amount of mineral lubricating oil and from about 1% to about 5%, of an oil-soluble linear hydrocarbon polymer containing on different carbon atoms of the linear hydrocarbon chain  $C_{8-20}$  alkyl groups and alkyl group containing on adjacent carbon atoms chlorine and



groups, the number of such units ranging from 100 to 800 and the molecular weight of the polymer being from about 1000 to about 500,000.

4. A mineral lubricating oil composition comprising a major amount of mineral lubricating oil and from about 1% to about 5% of an oil-soluble linear hydrocarbon polymer containing on different carbon atoms of the linear hydrocarbon chain  $C_{12-18}$  alkyl groups and alkyl groups containing an adjacent carbon atom and at least 4 carbons from the linear chain chlorine and



the number of such units ranging from 100 to 800 and the molecular weight of the polymer being from about 10,000 to about 500,000.

## References Cited in the file of this patent

## UNITED STATES PATENTS

|              |                 |               |
|--------------|-----------------|---------------|
| 2,236,168    | Dietrich        | Mar. 25, 1941 |
| 2,317,751    | Frolich et al.  | Apr. 27, 1943 |
| 2,479,450    | Young et al.    | Aug. 16, 1949 |
| 55 2,719,827 | Lowe            | Oct. 4, 1955  |
| 2,744,099    | Mitchell et al. | May 1, 1956   |
| 2,781,318    | Cyphers         | Feb. 12, 1957 |
| 2,800,450    | Bondi et al.    | July 23, 1957 |